# EUROPEAN PATENT SPECIFICATION

(11) **EP 2 191 921 B1**
(45) Date of publication and mention of the grant of the patent: **09.01.2013**
(21) Application number: 08020271.6
(22) Date of filing: 21.11.2008
(51) Int. Cl.: B22F 1/00, H01H 1/02, B22F 1/02, C22C 1/04, H01H 33/66

(54) **Process for producing a copper-chromium contact element for medium-voltage switchgear assemblies**
Verfahren zur Herstellung eines Kupfer-Chrom Kontaktelements für Schaltgetriebeanordnungen mittlerer Spannung
Procédé de production d'un élément de cuivre et chrome de contact pour des ensembles d'appareil de commutation à moyenne tension

(43) Date of publication of application: 02.06.2010
(73) Proprietor: ABB Technology AG, 8050 Zürich (CH)
(72) Inventor: Gentsch, Dietmar, Dr.-Ing., 40882 Ratingen (DE)
(74) Representative: Schmidt, Karl Michael

(56) References cited:
- EP-A2- 0 469 578
- EP-A2- 0 538 896
- DD-A1- 209 317
- US-A- 3 785 801
- US-A- 5 689 796
- US-A- 5 853 083

## Description

The invention relates to a process for producing a contact element for medium-voltage switchgear assemblies, and also to the contact element itself, in accordance with the preamble of claim 1.

Contact elements for medium-voltage switchgear assemblies are often produced by means of sintering processes. In this case, not only copper but also an alloy of copper and chromium is used for increasing the resistance to erosion. In the case of the sintering processes, it is known to press what are known as green compacts with near final dimensions in advance, and these green compacts are then annealed. Very large pressing forces are used during the pressing of the green compacts. In this case, the powder consisting of copper and chromium particles is placed in a mold and the pressing tool then compresses said particles with a high pressing force. It has been observed in this process that the extremely hard particles of the chromium powder have a considerable abrasive effect on the surface of the pressing tool. Even after a few pressing operations, this damage to the pressing tool leads to intolerable deviations in the final dimensions of the green compact and in the surface quality thereof. DD-209 317 discloses to produce contact elements for switches out of copper and copper-chromium powder in which the particles are rounded by milling.

The invention is therefore based on the object of improving a process for producing a contact element for medium-voltage switchgear assemblies, and also a contact element itself, in such a way as to considerably lessen the abrasive effect which occurs during operation when the contact element is finished, and therefore to make the contact element more durable during operation.

In the case of a process in accordance with claim 1, the set object is achieved according to the invention by means of the features of claim 1.

Further advantageous refinements are specified in dependent claim 2.

The essence of the invention in this case is that the chromium particles in the powder mixture are surface-rounded in advance. This considerably reduces the mechanically abrasive effect on the expensive pressing tool. In this case, however, the outer surface of the hard chromium particles can be rounded in different ways.

First the chromium particles are rounded mechanically in a mill, in particular in a ball mill. The chromium powder rounded in this way is then used, for its part, for the copper/chrominum powder mixture required for production.

In a further refinement, the already mechanically rounded chromium particles are provided with a copper layer. In detail, this means the following: this further copper coating is a further measure for the chromium particles which have already been mechanically rounded in advance.

During the heat treatment, heating is of course carried out up to that temperature at which the copper covers the chromium particles.

In a further advantageous refinement, it is provided that the process is carried out under vacuum, under a hydrogen atmosphere or under inert gas. Further oxidation processes are avoided in the process.

In terms of the contact element itself, the essence of the invention is that the chromium particles in the powder mixture have a surface-rounded structure before the pressing operation. This allows a low-abrasion, direct pressing operation with near final dimensions to be carried out using the pressing tool.

In the refinement, it is stated that the structure is provided mechanically by breaking the edges in a mill, and/or the chromium powder or the chromium powder particles mechanically rounded in this way is/are rounded by vaporizing with copper. This results in a homogeneous, high-quality green compact, in the case of which the pressing tool can operate with considerably less abrasion.

Since the process for pressing green compacts is also largely known for contact elements, no further explanation is required here.

The figure therefore merely shows an example of the microstructure of chromium powder particles as are used for this process.

A first illustration shows a chromium particle which has sharp edges per se. In this case, this particle is provided with a copper layer in the manner described, and the surface of the resulting copper-coated chromium particle is therefore rounded in this way.

The chromium particles are mechanically rounded in, for example, a ball mill. In this case, the chromium particles are additionally coated with copper. This then no longer only has the purpose of rounding, but also producing a copper/chromium alloy which is homogeneous as a result.

The coating operation takes place by means of vaporizing, or by layering copper and chromium powder without preceding mechanical pressure, and thermal tempering to a temperature at which copper powder melts or vaporizes and therefore coats the chromium powder.

It is easily possible to subsequently mill the mixture as it is not pressed. The powder obtained is then the starting material for filling a pressing mold and for the production of a green compact.

The figure therefore firstly shows the edged chromium particle 1.
The original shape of the chromium particle 1 has sharp edges and is therefore firstly rounded in a mill. It is then coated with copper, as described above.

## Claims

1. A process for producing a contact element for a medium-voltage switchgear assembly, in which a green compact is produced by pressing a powder consisting of a copper/chromium mixture, which is then sintered,
wherein the chromium particles in the powder mixture are surface-rounded in advance, by being rounded mechanically in a mill, in particular in a ball mill, and the already mechanically rounded chromium particles are provided with a copper layer, and the coating operation is done by means of vaporizing, or by layering copper and chromium powder without preceding mechanical pressure, and thermal tempering to a temperature at which copper powder melts or vaporizes and therefore coats the chromium powder.

2. The process as claimed in claim 1,
**wherein**
the process is carried out under vacuum, under a hydrogen atmosphere or under inert gas.

## Patentansprüche

1. Prozess zum Herstellen eines Kontaktelements für eine Mittelspannungs-Schaltanlagenbaugruppe, wobei ein grüner Kompaktkörper hergestellt wird, indem ein aus einem Kupfer-Chrom-Gemisch bestehendes Pulver gepresst wird, das anschließend gesintert wird,
wobei die Chrompartikel in dem Pulvergemisch zuvor oberflächengerundet werden, indem sie mechanisch in einer Mühle, insbesondere einer Kugelmühle, gerundet werden, und die bereits mechanisch gerundeten Chrompartikel mit einer Kupferschicht überzogen werden, und der Beschichtungsvorgang mittels Aufdampfen oder durch Aufschichten von Kupfer- und Chrompulver ohne vorausgehenden mechanischen Druck und durch thermisches Tempern auf eine Temperatur, bei der Kupferpulver schmilzt oder verdampft und dadurch das Chrompulver beschichtet, ausgeführt wird.

2. Prozess nach Anspruch 1, wobei der Prozess unter Vakuum, unter einer Wasserstoffatmosphäre oder unter Inertgas ausgeführt wird.

## Revendications

1. Procédé de production d'un élément de contact pour un ensemble appareillage de commutation moyenne tension, dans lequel un comprimé cru est produit en comprimant une poudre constituée d'un mélange cuivre/chrome, laquelle est ensuite frittée, dans lequel les particules de chrome dans le mélange de poudres sont arrondies en surface à l'avance, en étant arrondies mécaniquement dans un broyeur, en particulier dans un broyeur à boulets, et les particules de chrome déjà arrondies mécaniquement sont recouvertes d'une couche de cuivre, l'opération de revêtement étant réalisée au moyen d'une vaporisation, ou par superposition de la poudre de cuivre et de chrome sans pression mécanique préalable, et revenu thermique à une température à laquelle la poudre de cuivre fond ou se vaporise et par conséquent recouvre la poudre de chrome.

2. Procédé selon la revendication 1, le procédé étant mis en oeuvre sous vide, sous une atmosphère d'hydrogène ou sous gaz inerte.
